

# UNITED STATES PATENT OFFICE.

FREDERICK WILLIAM FLETCHER, OF HELPSTON, MARKET DEEPING, ENGLAND, ASSIGNOR  
OF ONE-HALF TO LIONEL WILLIAM JOHN DIGBY, OF HAYCOCK, WANSFORD, ENGLAND.

## ALLOY.

No. 867,194.

Specification of Letters Patent.

Patented Sept. 24, 1907.

Application filed July 20, 1906. Serial No. 327,085.

To all whom it may concern:

Be it known that FREDERICK WILLIAM FLETCHER, a subject of the King of Great Britain, residing at Helpston, Market Deeping, Lincolnshire, England, has invented certain new and useful Improvements in Alloys, of which the following is a specification.

The object of this invention is to manufacture a metallic alloy.

For the purpose of this invention, I take aluminium, gun metal (preferably soft formed from 90 parts of copper and 10 parts of tin) and white metal formed from a mixture of 6 parts tin with one part copper admixed with a mixture of 6 parts tin and one part of antimony in or about the following proportions:

15                   Aluminium = 30 lbs.  
                      Gun metal = 1 lb.  
                      White metal =  $\frac{1}{4}$  lb.

and melt them together, stirring the mass after becoming fluid until thoroughly amalgamated.

20                   I cast the metal into molds in strip form to form in-

gots for after use in making of articles in any well known way.

What I claim and desire to secure by Letters Patent is:—

1. A metallic alloy for shoes of beasts of burden, consisting of aluminium, gun metal (formed from a mixture of 90 parts of copper and 10 parts of tin), and white metal (formed from a mixture of 6 parts tin with 1 part copper admixed with a mixture of 6 parts tin and 1 part antimony) melted and alloyed together in or about the following proportions, aluminium 30 lbs., gun metal 1 lb., white metal  $\frac{1}{4}$  lb., substantially as set forth.

2. A metallic alloy consisting of aluminium, gun metal and white metal.

3. A metallic alloy consisting of thirty pounds of aluminium, one pound of gun metal, one-quarter pound of white metal.

In testimony whereof I have hereunto set my hand in presence of two subscribing witnesses.

FREDERICK WILLIAM FLETCHER.

Witnesses:

RICHARD CORE GARDNER,  
LYNWOOD FERDINAND GARDNER.